

## UNITED STATES PATENT OFFICE.

DANIEL BLUMENKRON, OF PUEBLA, MEXICO.

## MANUFACTURE OF MATCHES.

SPECIFICATION forming part of Letters Patent No. 242,427, dated June 7, 1881.

Application filed July 6, 1880. (Specimen.) Patented in Mexico October 8, 1879.

*To all whom it may concern:*

Be it known that I, DANIEL BLUMENKRON, a citizen of the United States, residing in the city of Puebla, State of Puebla, and Republic of Mexico, have invented certain new and useful Improvements in the Process and Compound for Manufacturing Matches; and I do hereby declare that the following is a full, clear, and exact description of the same, which will enable others skilled in the art to which it appertains to make and use the same.

The object of my invention is to produce a match inodorous, combustible, but not explosive, and impervious to air or water.

To carry my invention into effect, I take of bleached cotton yarn a number of strands, according to the size of the match desired. These strands are wound upon a reel, and having prepared an oval-shaped apparatus adapted to the purpose having a false bottom, the upper containing a mixture of sixty-two and a half (62 $\frac{1}{2}$ ) parts of stearine and four (4) parts of gum-dammar, and the lower or false bottom containing water heated to a temperature sufficient to retain the above mixture in a liquid state and of the consistency required, the strands are then unwound from the reel and allowed to pass through the above mixture several times until they have absorbed a sufficient quantity to give them the required thickness. They are then passed through a perforated steel mold-board, which gives them the necessary polish and uniformity. These strands, in combination with the above composition, form the body or stem of the match, which is then passed through an ordinary cutter, which divides it into the required lengths. These pieces are then transferred to a press, grooved to suit their size. A bath is then prepared of the following ingredients, to form the head or combustible portion of the match: red lead or minium, nine and twelve-sixteenths parts; nitric acid, (90° Fahrenheit,) five parts. This combination is then subjected to the action of heat, by means of which the first is transformed, under the influence of the second, into oxide of lead, which oxidizes readily, and thus facilitates the combustion of the phosphorus. I then dissolve two and seven-sixteenths pounds gum-arabic (senegal) in two and a half pounds water. Once dissolved, I

place the solution in a suitable tin vessel, with two pounds five and one-half ounces of phosphorus, which I place in a hot-water bath and stir continually until thoroughly mixed. To 55 this I add one ounce of sulphuret of antimony and the solution of red oxide of lead above referred to. The frame or press containing the stems or bodies of the matches is then dipped into this solution, thus forming the heads or 6 combustible property required. To render them water-proof they are allowed to remain in the press for four or five days, and when thoroughly dry they are again submitted to a bath in the following solution: I pulverize a 65 determined quantity of gum-shellac and spread it thinly in uncovered tin vessels adapted to the purpose in order to obtain the greatest possible evaporating-surface, which I place upon suitably-arranged iron bars in a furnace, and 70 submit the gum to a hot current of air for the space of five or six days, thus obtaining the complete oxidation of the gum and rendering it thoroughly soluble in alcohol.

I next prepare a solution of oxidized gum-shellac, one pound; alcohol, (90° Fahrenheit,) four pounds, by means of a hot-water bath, which, upon being filtered, gives as a result a thick claret-colored liquid, and is applied as a varnish to the head of the match and a small 80 portion of the stem by the following process: I place a sufficient quantity to a little more than cover the head of the match in a wooden vessel having a glass bottom, and placed exactly on a level, and then submerge the press containing the matches (already headed) for four or five seconds in the varnish, then removing them. I submit it then to a strong current of air, which thoroughly evaporates the alcohol and leaves the matches with a brilliant and 85 perfectly dry finish, thus rendering them water-proof; but, to make doubly sure, I again repeat the process and obtain a match that will resist the severest climate, and which, even if allowed to remain in water for several hours, 90 will ignite as readily and perfectly as before submitting it to this severe test.

Phosphorus, when it comes in contact with the atmosphere, produces a slow combustion, which at times is almost instantaneous, thus 100 being the cause of many fires; but as the head of my match is covered with a coating of var-

nish, this danger is obviated, for the reason that combustion cannot take place unless the match comes in direct contact with a surface sufficiently rough to remove this coating.

5 Although phosphoric vapors have no deleterious effect upon the human system, they are extremely disagreeable and offensive; but by combining with phosphorus the ingredients before described these objections are removed 10 and an inodorous match produced. Furthermore, these ingredients are harmless and the match non-explosive, which is not the case with the ordinary parlor-match now in common use.

What I claim, and desire to secure by Letters Patent, is—

1. A compound for matches, consisting of red oxide of lead, phosphorus, sulphuret of antimony, and a gummy vehicle for the same, in substantially the proportion hereinbefore set forth.

2. A water and air proof match having stem consisting of strands of cotton saturated and coated with a translucent inflammable water and air proof solution, and a head polished and waterproofed with an alcohol lac varnish, 25 as shown.

DANIEL BLUMENKRON.

Witnesses:

J. H. COYNE,  
J. B. WHITING.